

## UNITED STATES PATENT OFFICE

BORIS N. LOUGOVY, OF MONTCLAIR, NEW JERSEY, ASSIGNOR TO ELLIS-FOSTER COMPANY, OF MONTCLAIR, NEW JERSEY, A CORPORATION OF NEW JERSEY

## FLOOR RUG AND PROCESS OF MAKING SAME

No Drawing.

Application filed December 13, 1926. Serial No. 154,655.

This invention relates to floor coverings or floor rugs and to the process of making same, and relates in particular to such products prepared with the aid of nitrocellulose plastic compositions or equivalent material.

The preferred form of the present invention is that which involves sheeting onto a supporting web, for example, paper, a plastic composition containing a binder of nitrocellulose or cellulose acetate, cellulose ethers, and the like. In fact, the composition is not restricted to the cellulose esters mentioned, but may include others of an appropriate character. Mixtures of such cellulose esters or of these ethers and esters sometimes may be utilized.

Besides paper, other substances such as cloth, burlap, and the like, may be employed in carrying out my invention. Preferably, however, I employ a waterproof backing or support for the tread. For example, I may use what is known as saturated felt, that is, absorbent paper material impregnated with a soft asphaltic material affording a cushioning effect under the foot. In the preferred form of the invention, however, I use a waxed paper which is quite water resistant and which may be white or light colored instead of black as is the case with the saturated felt. The black color is disadvantageous in preparing certain types of light colored products and for other reasons.

It has been assumed that wax and nitrocellulose repel one another and therefore it would be the assumption that sheeting the nitrocellulose composition onto a well-waxed paper would not yield a tread of a sufficiently adherent character. I have found, however, that even though the paper contains an unnecessarily high proportion of wax from the waterproof standpoint, nevertheless, good adhesion between the tread and backing results.

45 In one form of the process I convert the

plastic tread material into a porous product having a notable degree of cushioning effect. This is preferably accomplished by the expansion of volatile solvents present in the soft plastic mass, all as will be more fully 50 hereinafter described in the illustrative example:

Filling material such as ground cork, wood fibre or pulp, ground wood or wood flour, linters, cotton flock, and the like, may be used as 55 filling material. Preferably I employ in the filler a variable proportion of vegetable ivory waste, obtained from button manufacturers. This may be secured in the form of a powder or fine shavings. Its presence in the tread composition tends to decrease inflammability without making too dense and hard a surface. Moreover, the presence of vegetable ivory results in a surface which exhibits 60 a good finish. Vegetable ivory sawdust, also appears to improve the sheeting of the composition onto the backing.

I may employ various forms of nitrocellulose, including grades of high and low viscosity.

70 Gelatinized nitrocellulose is desirable and preferably I employ at least a substantial proportion of scrap celluloid. In such material I have available a percentage of camphor or other plasticizers, together with antacids. The celluloid obtained by stripping the emulsion from spent moving picture films may be 75 employed to advantage. With this material, I may, if desired, add some fresh celluloid nitrocellulose, or may introduce low viscosity nitrocellulose. In general, however, I prefer the high viscosity nitrocellulose of the nature of celluloid stock, as it enables sheeting to be carried out to better advantage. The employment of aged celluloid such as is obtainable 80 in the form of celluloid scrap or film is desirable in making floor covering of the present invention.

An illustration involving the employment 90

of the preferred form of cellulose derivative is the following:

|                                  | Parts by weight |
|----------------------------------|-----------------|
| Cleaned moving picture film      | 200             |
| 5 Acetone                        | 300             |
| Benzol                           | 150             |
| Tricresyl phosphate              | 130             |
| Blown castor oil                 | 130             |
| Denatured alcohol                | 50              |
| 10 Paraffin wax                  | 10              |
| Benzoic phthalic glyceride resin | 60              |
| Rosin                            | 40              |

The film was dissolved in 200 parts of acetone and agitated in a Werner Pfleiderer mixer. The plasticizing and softening agents were added and a solution of the synthetic resin and the rosin carrying the wax was made in a mixture of the alcohol, benzol, and the 20 remainder of the acetone. This solution is turbid. This composition was thoroughly incorporated and to it was added:

|                              | Parts |
|------------------------------|-------|
| Vegetable sawdust            | 130   |
| 25 Wood flour                | 100   |
| Perhydrated calcium sulphate | 200   |
| Lithopone                    | 200   |
| Diphenylamine                | 5     |
| Pigment                      | 3     |

30 The last mentioned ingredient is pigment of any special color desired in the final (coated) product.

When this had become thoroughly incorporated to a smooth plastic putty, the composition was sheeted onto a paper base containing paraffin wax. Four grades of waxed paper were employed. One of these contained wax incorporated as a wax emulsion added to the paper pulp in the beater engine. The 40 proportion of wax in this composition was low and it was not as waterproof as the paper material described below.

The adhesion of the tread to the surface was 45 excellent.

Three grades of paper were waxed by dipping into a bath of molten paraffin wax. One grade had 58 parts by weight of wax incorporated to 100 parts of paper. A second 50 grade had 65 parts wax and a third grade 79 parts. These papers were very waxy to the touch and a recognition of the characteristic qualities of nitrocellulose would suggest the impossibility of securing adherence. On 55 the contrary an entirely sufficient degree of adhesion was secured. In applying the plastic material to the paper I employed calendering rolls. To obtain a porous tread the sheeted material was allowed to form a skin over the 60 surface by brief exposure to the air and was then exposed to a temperature of about 70° C. for five minutes. This caused the solvent to expand and form a spongy layer between the paper and the surface of the tread. The 65 surface was practically free from visible

pores, but a cross section of the floor rug clearly showed the porous spongy character of the under portion of the tread. I found that it was desirable to pass the dried material through rolls either cold or hot, in order to level the surface. The bubbles forming beneath the surface in the mass of the material render the surface somewhat irregular. This irregularity may be desirable for some purposes, but to obtain a more conventional finish, it is desirable to press or roll the surface to eliminate such undulations or slight elevations. This treatment may be carried out before the tread composition is dried out thoroughly and then the floor covering may be exposed to a gradual heat extending up to, say, 70° C. Preferably, however, the final temperature is kept below the melting point of the paraffin wax waterproofing agent. If desired, other waxes, especially those of light color, may be used in place of paraffin, or in admixture with paraffin, to raise the melting point. Thus, bleached Montan wax, carnauba wax, etc., may be utilized. At first, there is a rather strong odor of camphor due to the presence of this material in the moving picture film employed. On exposure, the odor of camphor largely disappears so as not to be objectionable.

It should be noted that the formation of a good porous under-tread depends on forming a sufficiently strong surface film to prevent any substantial rupturing of the surface while sponge formation is in progress.

The benzoic phthalic glyceride resin employed above was made by heating a mixture of 59 parts phthalic anhydride, 49 parts benzoic acid and 47 parts glycerol in a kettle provided with an agitator and carrying the temperature to about 260° C.

Instead of the benzoic phthalic glyceride resin, I may, when such synthetic resins are desired, use, for example, cottonseed phthalic glyceride resin, or other similar corresponding products made from glycol or pentaerythritol, and so forth. Resins of this character have a striking compatibility with nitrocellulose. In place of rosin, other resins such as dammar, may be employed, or these natural resins or the natural resin may be omitted entirely. Again, a modified rosin, namely; ester gum, or rosin glyceride may be used in some cases. Other plasticizers such as dibutyl phthalate, diethyl phthalate, and the like, may be employed.

As a consequence of the foregoing disclosure it will be evident that various modifications may be employed such as varying the proportion of the ingredients or substituting equivalent ingredients, or omitting certain ingredients not required for the particular purpose in hand, and I do not wish to limit myself by such specific formula in any respect other than that it serves as an illustration.

70

75

85

90

95

100

105

110

115

120

125

130

appropriate for a broad comprehension of the present invention.

Another feature has been presented with especial reference to the appended claims is the employment of preferably a highly waxed paper as a backing for a nitrocellulose plastic or coating composition sheeted, coated or otherwise surfaced thereon; said paper preferably containing or carrying at least 5 per cent by weight (of the paper) as wax (paraffin, ceresin, Montan, wax substitutes, e. g., metallic stearates, and the like) and advantageously containing 10 to 50 per cent of wax, such that a nitrocellulose sheeting or coating composition would be expected to have greater or less repellent effect on this waxy surface; whereas an adherent tread or tread-surface results and the combined tread and waxed paper backing yields a floor covering of an integral character.

20 In such floor covering the ratio of thickness of paper to that of the tread may be varied. In some cases the paper may be thin and the tread relatively thick; in others, the tread may be a thin coating or veneer on a relatively thick paper backing.

What I claim is:—

1. A floor covering comprising a highly waxed paper support impregnated with a wax which is substantially free from dark color, such support carrying a nitrocellulose tread composition adherent thereto.

2. A floor covering comprising a highly waxed paper support having light colored paraffin as its principal waxy constituent carrying a spongy nitrocellulose tread composition adherent thereto.

3. A floor covering comprising a highly waxed paper support carrying a spongy nitrocellulose tread composition adherent thereto; said tread composition containing finely divided vegetable ivory.

4. Floor covering comprising a nitrocellulose tread composition directly attached to a backing of paper carrying at least 5 per cent of impregnated paraffin wax.

5. In the process of making floor coverings, the step which comprises sheeting a plastic nitrocellulose tread composition of a putty-like consistency containing volatile solvent, onto a heavily waxed paper backing and drying to form a flexible tread layer adherent to said backing.

6. A floor covering comprising a heavily waxed paper backing, and a nitrocellulose tread composition containing vegetable ivory, sheeted upon the paper backing.

7. A heavily waterproofed paper backing having sheeted thereon a vesiculated nitrocellulose tread composition containing nitrocellulose, a filler, a plasticizer, a resin and wax.

8. A method of making a floor covering comprising sheeting a nitrocellulose tread composition containing a volatile solvent

upon a heavily waterproofed backing, and evaporating the solvent under conditions to produce a vesiculated tread.

9. A method of making a floor covering which comprises sheeting a nitrocellulose tread composition containing a volatile solvent upon a heavily waterproofed backing, evaporating the solvent under conditions to produce a vesiculated tread, and smoothing the surface of the tread composition. 70

10. A floor covering comprising a nitrocellulose tread composition carried by a backing of paper containing at least 5% of a waterproofing wax composition. 75

11. A floor covering comprising a nitrocellulose tread composition sheeted upon a paper backing, the paper carrying from 10 to 50% of wax. 80

12. A floor covering comprising a highly waxed paper support carrying a nitrocellulose tread composition adherent thereto and sheeted thereupon. 85

13. A floor covering comprising a waxed paper backing and a porous nitrocellulose tread composition sheeted thereon. 90

14. A waterproof paper backing having sheeted thereon a porous and vesiculated nitrocellulose tread composition. 95

15. A floor covering comprising vesiculated nitrocellulose tread composition having a substantially non-vesiculated surface. 100

16. A floor covering comprising a waterproof paper support and adherent thereto a vesiculated nitrocellulose tread composition having a substantially non-vesiculated surface. 105

17. A floor covering comprising a waxed paper backing, and a nitrocellulose tread composition containing vegetable ivory, sheeted upon the paper backing. 110

18. A waterproof paper backing having sheeted thereon a vesiculated nitrocellulose tread composition containing nitrocellulose, a filler, a plasticizer, a resin and wax. 115

19. As an article of manufacture, a sheeted article carrying a vesiculated nitrocellulose coating. 120

20. A method of making a floor covering comprising sheeting a nitrocellulose tread composition containing a volatile solvent upon a backing, and evaporating the solvent under conditions to produce a vesiculated tread. 125

21. A method of making a floor covering which comprises sheeting a nitrocellulose tread composition containing a volatile solvent upon a backing, evaporating the solvent under conditions to produce a vesiculated tread, and smoothing the surface of the tread composition. 130

BORIS N. LOUGOVOY.